



chloride or sulfate. Examples of presently useful metal 1,1,1-tri- and 1,1,1,5,5,5 - hexafluoroacetylacetones include the copper, barium, manganese, cobalt and nickel tri- and hexafluoroacetylacetones.

Metal chelates of other fluorinated acyclic diketones which can be used as antioxidants include: manganese, cobalt or

cadmium chelate of 1,1,1-trifluoro-2,4-hexanedione, nickel chelate of 5,5,6,6,6-pentafluoro-2,4-hexanedione, aluminum chelate of 1,1,1,2,2-pentafluoro-3,5-heptanedione, copper chelate of 1,1,2,2,6,6,7,7-octafluoro-3,5-heptanedione, zirconium chelate of 1,1,1,2,2,6,6,7,7-decafluoro-3,5-octanedione, titanium chelate of 1,1,1-trifluoro-2,4-decanedione, cobalt chelate of 1,1,1-trifluoro-2,4-decanedione, tin chelate of 1,1,1,2,2,3,3,4,4,5,5,6,6-tridecafluoro-7,9-pentadecanedione, manganese chelate of 5,5,6,6,6-pentafluoro-2,4-hexanedione, iridium chelate of 1,1,1,2,2-pentafluoro-3-propyl-4,6-nonanedione, germainum chelate of 1,1,1,2,2-pentafluoro-3,5-heptanedione, and the like.

Another class of carbonyl compounds which serve as ligands for preparation of the presently useful metal chelates can be those in which R includes a ring containing conjugated unsaturation, either heterocyclic including O, S, or N as the hetero atom, or carbocyclic including aryl, alkaryl or aralkyl. For example, these radicals may be furyl, thiienyl, pyranyl, pyridyl, phenyl,  $\alpha$ - or  $\beta$ -naphthyl, tolyl, 3-butylphenyl, benzyl, etc. Examples of such chelates are chelates of aryl, alkaryl and aralkyl diketones such as:

cobalt chelate of 4,4,4-trifluoro-1-phenyl-1,3-butanedione, nickel chelate of 4,4,4-trifluoro-1-phenyl-1,3-butanedione, cobalt chelate of 5,5,5-trifluoro-1-phenyl-2,4-pentanedione, manganese chelate of 5,5,5-trifluoro-1-tolyl-2,4-pentanedione, nickel chelate of 4,4,5,5,5-pentafluoro-1-phenyl-1,3-butanedione, copper chelate of 5,5,5-trifluoro-1-phenyl-2,4-pentanedione, cobalt chelate of 4,4,4-trifluoro-1-xylyl-1,3-butanedione, copper chelate of 4,4,4-trifluoro-1- $\alpha$ -naphthyl-1,3-butanedione, barium chelate of 4,4,5,5,6,6,7,7-octafluoro-1-(m-propyl-phenyl)-1,3-heptanedione, cobalt chelate of 9,9,9-trifluoro-1-phenyl-1,3-nonenedione, manganese chelate of 1,1,1-trifluoro-6-phenyl-2,4-hexanedione, cobalt chelate of 5,5,6,6-tetrafluoro-1-(p-isopropylphenyl)-2,4-hexanedione and the like, as well as heterocyclic chelates such as copper chelate of 4,4,4-trifluoro-1-(2-thienyl)-1,3-butanedione, nickel chelate of 4,4,4-trifluoro-1-(2-thienyl)-1,3-butanedione, cobalt chelate of 4,4,4-trifluoro-1-(2-thienyl)-1,3-butanedione, copper chelate of 4,4,4-trifluoro-1-(2-furyl)-1,3-butanedione, nickel chelate of 4,4,4-trifluoro-1-(2-furyl)-1,3-butanedione, copper chelate of 4,4,4-trifluoro-1-(3-furyl)-1,3-butanedione, nickel chelate of 4,4,4-trifluoro-1,2-pyridyl-1,3-butanedione, zinc chelate of 4,4,5,5,5-pentafluoro-1-thienyl-1,3-butanedione,

aluminum chelate of 4,4,5,5-tetrafluoro-1-thienyl-1,3-butanedione, manganese chelate of 4,4,4-trifluoro-1,3-pyridyl-1,3-butanedione, cobalt chelate of 4,4,4-trifluoro-1,3-pyridyl-1,3-butane-dione, cobalt chelate of 5,5,5-trifluoro-1-thienyl-2,4-pentanedione, nickel chelate of 5,5,5-trifluoro-1-thienyl-2,4-pentanedione, cobalt chelate of 4,4,5,5,5-pentafluoro-1-benzothienyl-1,3-pentanedione, aluminum chelate of 5,5,5-trifluoro-1-pyranyl-2,4-pentanedione, chromium chelate of 7,7,7-trifluoro-1-thienyl-1,3-heptanedione, and so forth.

The carbonylic ligand can also be an acylacetate ester of the formula:



where R is a fluorinated alkyl radical as defined above, and R' is an alkyl hydrocarbon radical of from 1 to 6 carbon atoms. Chelates formed from the use of such acylacetate esters as illustrated by:

30 cobalt chelate of ethyl trifluoroacetoacetate, copper chelate of methyl trifluoroacetoacetate, mercury chelate of t-butyl trifluoroacetoacetate, nickel chelate of ethyl 4,4,5,5,5-pentafluoro-3-oxovaleric acid, rhenium chelate of hexyl 4,4,5,5,5-pentafluoro-3-oxo-35 valeric acid, aluminum chelate of ethyl 4,4,5,5,6,6,7,7,8,8-decafluoro-3-oxooctanoate, cobalt chelate of isopropyl 5,5,5-trifluoro-4,4-bis(trifluoromethyl)-3-oxovalerate, aluminum chelate of ethyl trifluoroacetoacetate, 40 manganese chelate of ethyl trifluoroacetoacetate, copper chelate of methyl 4,4,5,5,5-pentafluoro-3-oxovalerate, lead chelate of ethyl 8,8,8-trifluoro-3-oxooctanoate, cobalt chelate of ethyl 9,9,9-trifluoro-3-oxononanoate, and 45 so forth.

The antioxidant additive employed in the formulated fluids of this invention can consist of the metal fluorinated carbonyl compound alone or in combination with further oxidation-suppressing additives. It has been found that particularly effective suppression of the oxidative degradation of the present base stock blends is produced by combination of amines with the metal carbonyl compounds.

55 For the present purpose, useful amines contain at least 12 carbon atoms. They may be either aromatic or aliphatic and are usually secondary or tertiary amines. Presently useful aromatic amines include arylamines and arylidene amines wherein the benzene nuclei are attached to the amine nitrogen atoms either directly by a ring carbon atom or through a single aliphatic carbon atom. The amines contemplated herein are free of aliphatic (olefinic and acetylenic) unsaturation, contain from 12 to 36 carbon atoms, and consist of hydrocarbon radicals and amino 60 nitrogen atoms, which may or may not have oxy (oxygen joined to atoms selected from C and H) or thio (joined to 2 C atoms) radicals as substituents. Generally, the presently contemplated amines will include from 1 to 4 nitrogen, from 0 to 3 oxygen, and from 0 to 2 sulfur atoms.

65 Illustrative of presently useful aromatic amines are aryl amines such as naphthylamine ( $\alpha$  or  $\beta$ ), naphthylene-diamine, 4-aminobiphenyl, 2-aminobiphenyl, 4-aminobiphenyl, diphenylamine, 4-aminodiphenylamine, N-phenyl-phenylenediamine, N-ethyl- $\alpha$ -naphthylamine, 2,4-diamino-

diphenylamine, 1,2-diphenylethylenediamine, N-benzyl-aniline, methylenedianiline, 1-aminoanthracene, 1-amino-phenanthrene, di-o-tolylamine, 4-dimethylaminodiphenyl-amine, N,N'-diphenylethylenediamine, o-ditoluidine (3,3-diamino-4,4-dimethylbiphenyl), N-phenyl- $\alpha$ -naphthyl-amine, N-phenyl- $\beta$ -naphthylamine, N-cyclohexyl- $\alpha$ -naphthylamine (or  $\beta$ ), N-p-tolyl- $\beta$ -naphthylamine, triphenyl-amine, N,N'-diphenyl-p-phenylenediamine, di- $\alpha$ -naphthyl-amine, di- $\beta$ -naphthylamine, triphenylamine, dibiphenyl-amine, N,N'-diphenylbenzidine, p-aminophenyltriphenyl-methane, N,N'-dinaphthylmethylenediamine, N,N'-dinaphthyl-p-phenylenediamine, N-[(1-aminocyclohexyl)methyl]-N'-phenyl-p-phenylenediamine, acridine, phenothiazine, and so forth.

Exemplary of presently useful arylidene amines are

N,N-dibenzylidene-p-phenylenediamine,  
N,N'-bis(2,3-dimethylbenzylidene)-p-phenylenediamine,  
N,N'-bis(2-hydroxybenzylidene)-p-phenylenediamine,  
N,N'-bis(2-ethoxybenzylidene)-p-phenylenediamine,  
N,N'-bis(2-hydroxybenzylidene)ethylenediamine,  
N,N'-bis(2-hydroxybenzylidene)-1,2-propylenediamine,  
N,N'-bis(2-hydroxybenzylidene)-1,3-propylenediamine,  
N,N'-bis(3-ethoxy-4-hydroxybenzylidene)-1,2-propyl-enediamine,  
N,N'-bis(2-hydroxy-4-methylbenzylidene)-p-phenyl-enediamine,  
N-3-methylbenzylidene-3-octylaniline,  
N-2-hydroxybenzylidene-4-hexadecylaniline,  
N,N'-bis(3,4-methylenedioxybenzylidene)-p-phenyl-enediamine,  
N,N'-bis((2,3-dimethoxybenzylidene)-p-phenylene-diamine,  
N,N'-bis(2-methoxybenzylidene)-p-phenylenediamine,  
N,N'-bis(2-hydroxybenzylidene)-o-phenylenediamine,  
N,N'-bis(3,4-methylenedioxybenzylidene)-p-phenyl-enediamine,  
N,N'-bis(3-ethoxy-4-hydroxybenzylidene)-p-phenyl-enediamine,  
N-(3-ethoxy-4-hydroxybenzylidene)-4-dodecylaniline,  
N,N'-bis(4-phenoxybenzylidene)-p-phenylenediamine,  
N,N'-dibenzylidene-1,2-diphenylethylenediamine, and the like,

Exemplary of presently useful aliphatic amines are, for example, N,N-dimethyloctadecylamine, N,N-diethyl-octadecylamine, N,N-dihexyloctadecylamine, N,N-dimethylhexadecylamine, N,N-dimethylleicosylamine, N,N-dibutylhexadecylamine, N,N-dimethyldecylamine, trihexadecylamine, N,N-dimethyldecylamine, trinonylamine, N-ethyl-N-methylhexadecylamine, N-butyl-N-propyloctadecylamine, and so forth.

To provide the fluid compositions of this invention, the metal fluorinated chelates of the nature stated above are combined, with or without addition of an amine, with a base fluid. These fluid compositions can be used for operation and lubrication of the moving parts of mechanisms operating in temperature ranges of 400° F. to 700° F. and up to 1000° F.

A particularly advantageous base fluid for use in mechanisms operating at 400° F. to 700° F. comprises the polyphenyl ethers. The polyphenyl ethers employed in the composition of this invention have from 3 to 7 benzene rings and from 1 to 6 oxygen atoms joining the benzene rings in chains as ether linkages. One or more of these benzene rings may carry hydrocarbyl substituents, which, for thermal stability, must be free of CH<sub>2</sub> and aliphatic CH. Thus, preferred aliphatic substituents are lower saturated hydrocarbon radicals (1 to 6 carbon atoms) like methyl and tertiarybutyl, and preferred aromatic substituents are aryl radicals like phenyl, tolyl, t-butylphenyl and  $\alpha$ -cumyl. Benzene rings supplied in the hydrocarbyl substituent contribute to the total number of benzene rings in the molecule.

Exemplary of the polyphenyl ethers containing

aliphatic carbon which are suitable for base fluids are 3-ring polyphenyl ethers like 1-(p-methylphenoxy)-4-phenoxylbenzene and 2,4-diphenoxyl-1-methylbenzene, 4-ring polyphenyl ethers like bis[p-(p-methylphenoxy)-phenyl]ether and bis[(p-tert-butylphenoxy)-phenyl]ether, and so forth. Polyphenyl ethers consisting exclusively of benzene rings and including ether oxygen atoms linking said rings are exemplified by the triphenoxy benzenes and aryl-substituted polyphenyl ethers such as biphenyl phenoxy-phenyl ether, biphenyloxyphenyl phenoxyphenyl ether, biphenyl ether, dibiphenyloxybenzene, bis(biphenyl-oxyphenyl)ether, and the like.

A preferred class of the polyphenyl ethers are those consisting of benzene rings joined in a chain by oxygen atoms as ether linkages between each ring, of the formula C<sub>6</sub>H<sub>5</sub>O-(C<sub>6</sub>H<sub>4</sub>O-)<sub>n</sub>-C<sub>6</sub>H<sub>5</sub> where n is an integer of from 1 to 5. Example of these polyphenyl ethers are the bis(phenoxyphenyl) ethers (4 benzene rings joined in a chain by 3 oxygen atoms), illustrative of which is bis(m-phenoxyphenyl)ether. The bis(phenoxyphenyl) benzenes, which are particularly valuable, are illustrated by m-bis(m-phenoxyphenyl)benzene, m-bis(p-phenoxy-phenyl)benzene, o-bis(o-phenoxyphenyl)benzene, and so forth. Further, the polyphenyl ethers contemplated herein include the bis(phenoxyphenoxyphenyl) ethers such as bis[bis[m-(m-phenoxyphenyl)phenyl]ether, bis[p-(p-phenoxyphenyl)phenyl]ether, and m-(m-phenoxyphenyl)phenyl m-(o-phenoxyphenyl)phenyl ether and the bis(phenoxyphenoxyphenyl) benzenes such as m-bis[m-(m-phenoxyphenyl)phenoxy]benzene, p-bis[p-(m-phenoxyphenyl)phenoxy]benzene and m-bis[m-(p-phenoxyphenyl)phenoxy]benzene.

The preferred polyphenyl ethers are those having all their ether linkages in the meta-positions, because of their wide liquid range and high thermal stability. Mixtures of the polyphenyl ethers, either of isomers or of homologs, can also advantageously be used in some applications, especially where particular properties such as lower solidification points are required. Mixtures of polyphenyl ethers in which the nonterminal phenylene rings are linked through oxygen atoms in the meta and para positions have been found to be particularly suitable to provide compositions with wide liquid ranges. An example of such preferred polyphenyl ether compositions are those containing, in percent by weight, from about 0 to 6% of o-bis(m-phenoxyphenyl)benzene (1), about 40 to 85% of m-bis(m-phenoxyphenyl)benzene (2), about 0 to 40% of m-[m-phenoxyphenyl](p-phenoxyphenyl)benzene (3), about 0 to 12% of p-bis(m-phenoxyphenyl)benzene (4), about 0 to 10% of p-[p-phenoxyphenyl](m-phenoxyphenyl)benzene (5), and about 0 to 6% of m-bis(p-phenoxyphenyl)benzene (6). Typical compositions of such preferred compositions are listed below. The number in parentheses refers to the compound mentioned above having the same number thereafter.

|            | Compositions,<br>Percent by weight of<br>components |    |    |      |
|------------|-----------------------------------------------------|----|----|------|
|            | A                                                   | B  | C  | D    |
| Component: |                                                     |    |    |      |
| (1)-----   | 0                                                   | 6  | 5  | 4.5  |
| (2)-----   | 63                                                  | 82 | 80 | 43.5 |
| (3)-----   | 31                                                  | 0  | 4  | 40   |
| (4)-----   | 0                                                   | 12 | 11 | 4    |
| (5)-----   | 0                                                   | 0  | 0  | 8    |
| (6)-----   | 6                                                   | 0  | 0  | 0    |

The above-discussed polyphenyl ether base fluids are especially thermally stable members of the class of base fluids which are aromatic rings connected by oxygen atoms.

A closely related class of base fluids are the all meta

linked polyphenyl thioethers represented by the following structure:



wherein  $n$  is a whole number from 1 to 3, polyphenyl thioethers represented by the following structure:



and phenyl mercapto biphenyls represented by the structure:



wherein  $x$  and  $y$  are whole numbers from 1 to 3 and the sum of  $x$  and  $y$  is from 2 to 6.

Typical examples of the polyphenyl thioether are *m*-bis(phenylmercapto)benzene, *m*-bis(*m*-phenylmercapto-phenyl[mercapto])benzene, phenylmercapto biphenyl, *o*-bis(*o*-phenylmercaptophenyl)sulfide, *m*-bis(*p*-phenylmercaptophenyl)sulfide, 1,2,3; 1,2,4, or 1,3,5 tris(phenylmercapto)benzenes; 2,2' or 4,4' bis(phenylmercapto) biphenyl, *o*, *m*, or *p*-bis (*o*, *m*, or *p*-phenyl mercapto-phenylmercapto)benzene, or -bis (phenylmercapto)-ar'-(phenylmercapto)benzene, 2,2', 4,4'-tetra and 2,2', 3,3', 4,4'-hexa (phenylmercapto)biphenyls.

Also useful as functional fluids in this invention are mixed polyphenyl ethers-thioethers corresponding to the formula:



wherein  $R$  is a phenyl group,  $R_1$  is a phenylene group and  $Y$  and  $Y_1$  are selected from the group consisting of O and S provided that at least one of  $Y$  and  $Y_1$  is S and one of  $Y$  and  $Y_1$  is O and  $n$  is a whole number of from 1-4. Examples of such mixed ether-thioethers are: 2 phenylmercapto - 4' - phenoxydiphenyl sulfide, 3 phenoxy - 4'-phenylmercapto diphenyl sulfide, 2,2' - bis(phenylmercapto)diphenyl ether, etc. The phenyl and phenylene groups of such compounds may contain substituents such as an alkyl of 1 to 4 carbon atoms, alkoxy of 1 to 4 carbon atoms; halogen and perfluoroalkyl of 1 to 4 carbon atoms. Examples are 3,3' - bis(xylylmercapto)diphenyl ether, 3,3' - bis(3-chlorophenylmercapto)diphenyl ether, 4,4' - bis(*m* - trifluoromethyl phenylmercapto)diphenyl ether, 3,4 - bis(*m* - isopropoxyphenylmercapto)diphenyl ether, 2-p-tolyloxy-3'-phenylmercapto diphenyl sulfide, etc.

The high temperature base fluids employed in the compositions of this invention can also comprise synthetic ester base fluids. These are fluids of lubricating viscosity and thermally stable to at least about 400° F., which are esters of alcohols containing at least 4 carbon atoms and which generally contain more than one ester group, and contain a total of at least 10 carbon atoms. They may be esters of polyhydric alcohols, of polybasic acids, or both.

The stated synthetic esters are generally aliphatic in nature, as distinguished from the essentially aromatic nature of the polyphenyl ethers, and their properties and

response to additives have correspondingly been found to be usually of a different kind. Unexpectedly, however, the presently contemplated metallic additives have also been found to provide significant improvement in the oxidation resistance of the stated ester type of base fluid. Ester fluids are illustrated by diesters of long chain ( $C_6$  and above) dicarboxylic acids like azelaic acid with long-chain branched primary alcohols of the  $C_4$  to  $C_{10}$  range; the esters of long chain ( $C_6$  and above) monobasic acids such as pelargonic acid with glycols such as polyethylene glycols; complex esters formed by linking dibasic acid half esters through a glycol such as dipropylene glycol, a polyethylene glycol of 200 molecular weight, and so forth. These methods of forming polyester type lubricant fluids can be combined and permuted, and different polyester products can be blended. Simple esters providing suitable fluids can be exemplified, for example, by bis(2-methylbutyl) sebacate, bis(1-methyl-4-ethyloctyl) sebacate, bis(2-ethylhexyl) sebacate, dipropylene glycol dipelargonate, the diesters of acids such as sebacic, azelaic and adipic acid with complex  $C_8-C_{10}$  primary branched chain alcohols such as those produced by the oxo process, polyethylene glycol 200 bis-(2-ethylhexyl sebacate), diisoamyl adipate, 1,6-hexamethylene glycol di(2-ethylhexanoate), bis(dimethylamyl) azelate and so forth.

Ester fluids with particularly good high temperature oxidation resistance are provided by neopentyl polyol esters. The alcohols from which these esters are derived have the carbon structure of neopentane, with a central carbon atom surrounded by 4 substituent carbon atoms. Included in the neophenyl polyols are neopentyl glycol, trimethylolethane, trimethylolpropane and pentaerythritol. Generally, the base fluids comprising neopentyl polyol esters are the esters with monocarboxylic acids. Such esters are generally more oxidatively and thermally stable than the dibasic acid esters. The useful esters of the neopentyl polyols include, for example, the esters of trimethylol propane, neopentyl glycol and pentaerythritol with normal, branched chain and mixed acids having chain lengths varying from  $C_6$  to  $C_{12}$ . Thus, an illustrative series of esters are trimethylolpropane tri-*n*-pelargonate, trimethylolpropane tricaprate, trimethylolpropane tricaprylate, the trimethylolpropane triester of mixed octanoates, and the like.

For further description of still other ester fluids adapted for use as lubricant base stocks and useful in the provisions of blends of this invention, reference may be made, for example, to the discussion in Gunderson et al., "Synthetic Lubricants" (Reinhold, 1962).

The base fluid in the present compositions may comprise polyphenyl ether, a polyphenyl thioether, a polyphenyl ether-thio-ether or a combination of two or more of the foregoing. Compositions comprising combinations of esters and the polyphenyl ethers have desirable fluidity at low temperatures. While various esters have been found to blend with the polyphenyl ethers to provide blends having thermal and oxidative stability approaching the stability of the polyphenyl ethers, especially valuable base fluids have been found to be provided by combinations of a polyphenyl ether with a neopentyl alcohol ester. These compositions possess both fluidity at low temperature and stability at elevated temperatures. The preferred polyphenyl ethers for use in this connection are the bis(phenoxyphenoxy)benzenes, of the composition  $C_6H_5O-(C_6H_4O-)_3-C_6H_5$  where each  $C_6H_5$  is a phenyl and each  $C_6H_4$  is a phenylene radical. Those with the ether linkages between benzene rings in meta positions, partly or wholly, are especially preferred. The stated neopentyl esters are esters of neopentyl alcohols such as pentaerythritol, trimethylolethane, trimethylolpropane and neopentyl alcohol with straight chain, branched chain and mixed  $C_5-C_{10}$  acids such as *n*-heptanoic and *neo*heptanoic acid. Compositions of the stated valuable nature are provided by combining 25-75 weight

percent of the ester base fluids with 75-25 weight percent of the polyphenyl ethers.

As noted hereinabove, antioxidant additives activity is usually not found to be general to different classes of lubricant base fluids. However, compositions comprising the presently employed chelates have unexpectedly been found to possess improved properties compared to the base stock alone with base oils of diverse kinds.

Thus, in its broadest aspects, this invention relates to functional fluid compositions in which the base stocks are those described above, or can be a lubricating oil, preferably an oil which is thermally stable up to about 500° F. Examples of such oils include, hydrocarbon oils, silicon-containing oils, fluorinated oils, and so forth.

Illustrative of hydrocarbon oil base fluids are the aromatic hydrocarbons, particularly condensed ring structures such as biphenyl, alkylbiphenyls such as mono- and diisopropylbiphenyl, and terphenyls, quaterphenyls, their alkyl derivatives such as dimethylterphenyl, and the like. Hydrogenated derivatives of these aromatic hydrocarbons, including alicyclic rings and alkylated alicyclic rings, can also be used. Mineral oils, paraffinic and naphthenic, can be provided with improved high temperature stability by super-refining. Super-refining is the removal or substantial reduction of the polar impurities, unsaturated and unstable hydrocarbon structures by exhaustive hydrogenation, severe acid treatment, adsorption, or a combination of these processes. Oxidation rates at 500° F. are approximately the same for the super-refined mineral oils as for the ester lubricants. Useful mineral oils are the petroleum products boiling above the kerosene range; a typical mineral oil base for extreme pressure lubrication will be characterized by a viscosity of 35-350 Saybolt Universal Seconds at 212° F., a viscosity index of -25 to +150 and a flash point of 275° to 600° F.

Silicon-based lubricant fluids are exemplified by silanes, such as n-dodecyl tri-n-decyl silane and diphenyl di-n-dodecyl silane; the silicone polymer fluids such as dimethyl silicone and methyl phenyl silicone polymers, and disiloxanes; and tetraalkyl orthosilicate esters such as di-tert-butyl di-2-ethylhexyl orthosilicate, 1,3-di-tert-butoxy-1,1,2,2-tetra-(2-pentoxy) disiloxane, tetra-(methylphenyl) silicate, tetraphenyl silicate, tetra(2-ethylhexyl) silicate, and so forth.

Illustrative of fluorine-containing base fluids are fluorinated esters like bis(perfluoroamyl) phthalate, bis(perfluorohexyl) 3-methylglutarate, and 1,1-H-nonafluoropentyl nonafluoropentanoate; and the polymers of chlorotrifluoroethylene, for example, with average molecular weights of about 500-1000, and so forth.

The compositions of this invention comprise a major proportion of the base fluid and a minor proportion of the metal chelate (and, when present, amine) additives. In general, the concentrations to be employed for effective improvement of the base fluid oxidative degradation resistance by the metal chelate and, when present, amine antioxidant compounds are between about 0.01% and 10%, individually or jointly, by weight of the fluid. Particular effective amounts depend on the nature of the individual additive and of the base fluid. To supply additive concentrates, adapted for later formulation of finished lubricant compositions, useful compositions may comprise up to about 1:1 weight ratio of the additives of this invention and the base fluid. In any case, at least an adjuvant amount sufficient to produce an improvement in the oxidation stability of the base fluid will be employed. Whether or not the desired antioxidant effect is obtained is readily determined by use of conventional testing procedures.

The compositions of this invention, in addition to the base fluid and the metal chelate compound, can additionally include further additives. For example, these can include sludge inhibitors and detergents such as the oil-

soluble petroleum sulfonates, to loosen and suspend products of decompositions and counteract their effect, viscosity index improvers, as exemplified by alkyl methacrylate polymers, pour point depressants, oiliness agents, anti-wear and lubricity agents, corrosion- and rust-inhibitors, anti-foam agents, and so forth.

The invention is illustrated but not limited by the following examples, in which the tests employed to determine the reported antioxidant effects of the additive compounds when employed with the base fluid are conducted as follows:

For determination of the antioxidant effect of the present additive compounds, air is bubbled through heated samples. The present change in (100° F.) viscosity from before to after oxidation is an index of antioxidant activity: desirably, the change is low. For a preliminary oxidation test, conditions employed are 450° F. temperature and a flow rate of 1 liter of air per hour, continued for 16 hours. Samples are run in the presence of metal wires (Fe, Ag, Cu, Al) as a check on the effect of such metals on oxidation temperature of 450° F. and in air flow rate of 5 liters per hour, continued for 24 hours.

#### EXAMPLE 1

This example illustrates use of metal fluorinated pentanedionate chelates as antioxidant additives for base fluids.

The ester base fluid used in the tests described below, identified as TMP, is trimethylolpropane trienanthate.

The polyphenyl ether base stock referred to in the following discussion is a bis(phenoxyphenoxy)benzene mixture of the composition: 65% m-bis(m-phenoxyphenoxy)benzene, 30% m-[ (m-phenoxyphenoxy) (p-phenoxyphenoxy)] benzene, 5% m-bis(p-phenoxyphenoxy)benzene.

Using the 16 hour, 1 liter/hour test described above, results obtained in TMP ester base fluids were as follows (results reported as average percent viscosity ( $\eta$ ) increase):

| Additive:             | Average percent increase |
|-----------------------|--------------------------|
| None                  | 48                       |
| Co(HFAA) <sub>2</sub> | 22                       |
| Co(TFAA) <sub>2</sub> | 20                       |
| Co(TTFA) <sub>2</sub> | 17                       |
| Co(ETFA) <sub>2</sub> | 43                       |
| Cu(HFAA) <sub>2</sub> | 33                       |
| Cu(TFAA) <sub>2</sub> | 26                       |
| Cu(ETFA) <sub>2</sub> | 37                       |
| Mn(HFAA) <sub>2</sub> | 30                       |
| Mn(TFAA) <sub>2</sub> | 39                       |
| Mn(TTFA) <sub>2</sub> | 37                       |
| Mn(ETFA) <sub>2</sub> | 36                       |

HFAA=hexafluoroacetylacetone

TFAA=trifluoroacetylacetone

TTFA=thenoyltrifluoroacetone (4,4,4 - trifluoro - 1 - 2 - thiienyl-1,3-butanedione

ETFA=ethyltrifluoroacetolacetate

Using the 24 hour, 5 liter per hour test described above, results obtained with the same ester base fluid were as follows:

| Additive              | Average percent $\eta$ increase |
|-----------------------|---------------------------------|
| None                  | 710                             |
| Co(TTFA) <sub>2</sub> | 250                             |
| Co(HFAA) <sub>2</sub> | 180                             |

In each of these tests little or no corrosion of the metal wires was observed.

#### EXAMPLE 2

This example illustrates use of the metal fluorinated carbonyl chelate additives of this invention in combination with secondary amines.

In the 16 hours, 1 liter/hour test described above, results were as follows for TMP ester:

| Metal additive:       | Amine additive | Average percent increase |
|-----------------------|----------------|--------------------------|
| None                  | None           | 48                       |
| Do                    | DOPA           | 28                       |
| Do                    | PANA           | 127                      |
| Ni(HFAA) <sub>2</sub> | DOPA           | 19                       |
| Ni(HFAA) <sub>2</sub> | PANA           | 20                       |
| Ni(TFAA) <sub>2</sub> | DOPA           | 23                       |
| Ni(TFAA) <sub>2</sub> | PANA           | 8                        |
| Ni(TTFA) <sub>2</sub> | DOPA           | 26                       |
| Ni(ETFA) <sub>2</sub> | PANA           | 14                       |
| Mn(TFAA) <sub>2</sub> | PANA           | 17                       |

<sup>1</sup> Filtered.

NOTE.—HFAA, TFAA, TTFA, ETFA: see Example 1; DOPA=di-octylphenylamine; PANA=phenyl- $\alpha$ -naphthylamine.

In the 24 hour, 5 liter/hour test, in the same ester base fluid, results obtained were:

| Metal additive:       | Amine additive | Average percent increase |
|-----------------------|----------------|--------------------------|
| None                  | None           | 710                      |
| Ni(HFAA) <sub>2</sub> | DOPA           | 270                      |

As in the previous example no corrosion of the metal wires was observed.

### EXAMPLE 3

This example illustrates improvement of the oxidation resistance of a base fluid by a metal fluorinated carbonyl chelate in combination with a tertiary amine.

With the test method described above, run for 16 hours at 1 liter/hour, the following results were obtained in TMP base stock.

| Metal Additive:       | Amine additive | Average percent increase |
|-----------------------|----------------|--------------------------|
| None                  | None           | 48                       |
| Do                    | $\phi_3N$      | 45                       |
| Do                    | DMODA          | 24                       |
| Co(HFAA) <sub>2</sub> | $\phi_3N$      | 13                       |
| Co(HFAA) <sub>2</sub> | DMODA          | 13                       |
| Cu(HFAA) <sub>2</sub> | $\phi_3N$      | 19                       |
| Mn(HFAA) <sub>2</sub> | DMODA          | 12                       |

<sup>1</sup> HFAA=hexafluoroacetylacetone.

$\phi_3N$ =triphenylamine; DMODA=dimethyloctadecyl amine ( $Me_2NCl_6H_{33}$ ).

At 24 hours, 5 liters/hour, in the same base stock results were as follows:

| Metal additive:       | Amine additive     | Average percent increase |
|-----------------------|--------------------|--------------------------|
| None                  | None               | 710                      |
| Co(HFAA) <sub>2</sub> | do                 | 200(220, 180)            |
| Co(HFAA) <sub>2</sub> | $\phi_3N$          | 70                       |
| Co(HFAA) <sub>2</sub> | DMODA              | 135                      |
| Co(HFAA) <sub>2</sub> | Acridine           | 65                       |
| Co(HFAA) <sub>2</sub> | DMODA and acridine | 20                       |

### EXAMPLE 4

This example describes preparation of the metal chelates. Melting points and colors of the chelates are presented in the table below.

(1) Hexafluoroacetylacetones.—With the exception of Al(HFAA)<sub>3</sub> and Zn(HFAA)<sub>2</sub>, the metal chelates are prepared by addition of hexafluoroacetylacetone to a stirred aqueous sodium acetate solution of the respective metal halides. The Zn(HFAA)<sub>2</sub> is prepared by addition of HFAA to an aqueous solution of zinc acetate and the Al(HFAA)<sub>3</sub> by addition of HFAA to an aqueous buffered suspension of aluminum hydroxide.

(2) Trifluoroacetylacetones.—The same general procedure described for the preparation of the hexafluoroacetylacetones is followed.

(3) Ethyl trifluoroacetoacetates.—With the exception of Al(ETFA)<sub>3</sub>, the same general procedure for preparing the hexafluoroacetyl- and trifluoroacetylacetones is followed. Al(ETFA)<sub>3</sub> is prepared in an aqueous sodium acetate buffered solution of aluminum nitrate.

(4) Thienoyl trifluoroacetonates.—The same general procedure used for preparing the metal chelates of the other ligands is followed except that 50% aqueous methanol is used as a solvent.

### 10 COLORS AND MELTING POINTS OF METAL CHELATES AND DERIVATIVES

| Chelate:               | Color           | Melting point, °C. |
|------------------------|-----------------|--------------------|
| Co(HFAA) <sub>2</sub>  | Orange-brown    | 192-194            |
| Ni(HFAA) <sub>2</sub>  | Aqua            | 208-210            |
| Fe(HFAA) <sub>3</sub>  | Red             | 46-47              |
| Cu(HFAA) <sub>2</sub>  | Green           | 117-118            |
| Mn(HFAA) <sub>2</sub>  | Yellow          | 158-160            |
| Ti(HFAA) <sub>4</sub>  | White           | 88-90              |
| Cr(HFAA) <sub>3</sub>  | Brown           | 111-114            |
| Al(HFAA) <sub>3</sub>  | White           | 88-89              |
| Zn(HFAA) <sub>2</sub>  | do              | 151-153            |
| Co(TFAA) <sub>2</sub>  | Pale orange     | 184-187            |
| Ni(TFAA) <sub>2</sub>  | Pale blue-green | 255-280            |
| Fe(TFAA) <sub>3</sub>  | Orange          | 114-116            |
| Cu(TFAA) <sub>2</sub>  | Blue green      | 196-197            |
| Mn(TFAA) <sub>2</sub>  | Yellow          | 138-141            |
| Cr(TFAA) <sub>3</sub>  | Brown           | 126-132            |
| Co(ETAA) <sub>2</sub>  | Orange          |                    |
| Ni(ETAA) <sub>2</sub>  | Green           | 205-207            |
| Fe(ETAA) <sub>3</sub>  | Orange-red      | 92, 5-93           |
| Cu(ETFAA) <sub>2</sub> | Pale blue-green |                    |
| Mn(ETFAA) <sub>2</sub> | White           | 86-88              |
| Al(ETFAA) <sub>3</sub> | do              | 96-97              |
| Co(TTFA) <sub>2</sub>  | Orange          | 192-195            |
| Ni(TTFA) <sub>2</sub>  | Light green     | >265               |
| Cu(TTFA) <sub>2</sub>  | Green           | 238-239            |
| Mn(TTFA) <sub>2</sub>  | Yellow          | 185-190            |
| Fe(TTFA) <sub>3</sub>  | Red             | 160-162            |
| Cr(TTFA) <sub>3</sub>  | Green-brown     | ( <sup>2</sup> )   |
| Al(TTFA) <sub>3</sub>  | White           | 205-206            |

<sup>1</sup> Decomposes.

<sup>2</sup> Wide range.

### EXAMPLE 5

This example describes utilization of some of the present additives in other base stocks.

Compositions are prepared by combining base fluids, metal fluorinated chelates and amines as stated below.

| Base Stock                    | Metal chelate         | Amine     |
|-------------------------------|-----------------------|-----------|
| Polyphenyl ether <sup>1</sup> | Fe(HFAA) <sub>3</sub> | $\phi_3N$ |
| Diocyl sebacate               | Ti(HFAA) <sub>4</sub> | PANA.     |
| Super-refined mineral oil     | Cr(TFAA) <sub>3</sub> | DOPA.     |
| Tetraoctyl silicate           | Al(TTAA) <sub>3</sub> | DMODA.    |
| Bis(perfluoroamyl)phthalate   | Zn(HFAA) <sub>2</sub> | Acridine. |

<sup>1</sup> The mixture described in Example 1.

The amine additives are present in concentrations of 0 to 1%, and the metal chelates, in concentrations of 1%, by weight of the base fluid. The compositions have improved oxidation stability compared to the base fluids and do not corrode metal wires used in the oxidation stability tests.

The compositions of this invention are particularly valuable as high temperature lubricants since they are stable to both thermal and oxidative degradation when used in lubricate moving parts subject to elevated temperatures. Most of the compositions will operate for extended periods at temperatures of 400-500° F. without failure and many will operate for somewhat shorter periods of time at temperatures up to nearly 1000° F.

The compositions, moreover, are valuable as force transmitting media for translating the movement of one or more mechanical means to one or more movable devices. For instance, they may be used in hydraulic brake devices in which the movement of a piston in a master cylinder is transmitted by the fluid to one or more brake actuating devices. They also are useful in hydraulic systems actuated by a pump, e.g., in a fluid motor comprising a constant- or variable-discharge piston pump which is caused to rotate by the pressure of the fluid of the system.

For use in a conventional automatic transmission, the presently provided functional fluid compositions are contained in the outer casing of the transmission device, which casing is attached to the usual engine crankshaft and flywheel and rotates therewith. Within the fluid is a coupling comprising an impeller connected to said casing and a turbine which is connected to the drive shaft of the vehicle. The turbine is driven by the motion of the fluid in response to the rotation of the impeller, as the casing to which the impeller is attached is actuated by the crankshaft and flywheel.

In all of these applications the fluid compositions of this invention are particularly useful because of their unusual stability to oxidative degradation, their thermal stability and their lubricating properties which render the system self-lubricating.

While the invention has been described with particular reference to various specific preferred embodiments thereof, it is to be appreciated that modification and variations can be made without departing from the scope of the invention, which is limited only as defined in the appended claims.

I claim:

1. A functional fluid composition consisting essentially of a fluid neopentyl polyol ester or a blend of said ester containing about 25-75 weight percent ester and a fluid polyphenyl ether, a fluid polyphenyl thioether, a fluid polyphenyl ether-thio-ether or ether mixture, and an amount, sufficient to stabilize said ester against oxidation, of a chelate of cobalt with hexafluoroacetylacetone.

2. A functional fluid composition consisting essentially of a fluid neopentyl polyol ester or a blend of said ester containing about 25-75 weight percent ester and a fluid polyphenyl ether, a fluid polyphenyl thioether, a fluid polyphenyl ether-thio-ether or ether mixture, and, an amount, sufficient to stabilize said ester against oxidation, of a chelate of nickel with hexafluoroacetylacetone.

3. A functional fluid composition consisting essentially of a fluid neopentyl polyol ester or a blend of said ester containing about 25-75 weight percent ester and fluid

5

polyphenyl ether, a fluid polyphenyl thioether, a fluid polyphenyl ether-thio-ether or ether mixture, and an amount, sufficient to stabilize said ester against oxidation, of triphenyl amine and cobalt bis hexafluoroacetylacetone.

10

4. A functional fluid composition consisting essentially of a fluid neopentyl polyol ester or a blend of said ester containing about 25-75 weight percent ester and a fluid polyphenyl ether, a fluid polyphenyl thioether, a fluid polyphenyl ether-thio-ether or ether mixture, and an amount, sufficient to stabilize said ester against oxidation, of acridine and cobalt bis hexafluoroacetylacetone.

15

5. A composition consisting essentially of a mixture of bis(phenoxyphenoxy)benzenes and trimethylolpropane trienanthate and an antioxidant additive consisting essentially of cobalt (II) chelate with hexafluoroacetyl acetone.

20

6. A composition consisting essentially of a mixture of bis(phenoxyphenoxy)benzenes and trimethylolpropane trienanthate and an antioxidant additive consisting essentially of an amine chosen from the group consisting of aryl amine, arylidene amine and aliphatic amine, said amine containing from 12-36 carbon atoms, from 1-4 nitrogen atoms, from 0-3 oxygen atoms and from 0-2 sulfur atoms, useful as an antioxidant in an ester-based functional fluid and nickel (II) chelate with hexafluoroacetylacetone in an amount sufficient to stabilize said composition against oxidation.

25

#### References Cited

#### UNITED STATES PATENTS

2,795,549 6/1957 Abbott et al.  
3,360,467 12/1967 McHugh et al.

35 MAYER WEINBLATT, Primary Examiner

D. SILVERSTEIN, Assistant Examiner

U.S. CL. X.R.

40 252—74, 400, 402, 403, 407